

## UNITED STATES PATENT OFFICE

LAWRENCE BRADSHAW AND HENRY V. DUNHAM, OF BAINBRIDGE, NEW YORK, AS-SIGNORS, BY MESNE ASSIGNMENTS, TO THE CASEIN MANUFACTURING COMPANY OF AMERICA, INC., OF NEW YORK, N. Y., A CORPORATION OF DELAWARE

PROCESS OF MAKING SLOW-SETTING CASEIN GLUE, AND DRY BASE FOR USE IN SUCH PROCESSES

No Drawing.

Application filed May 19, 1926. Serial No. 110,298.

This invention has for its object improvements in casein glues and particularly waterproof casein glues or adhesives.

It is well known that glues and adhesive compositions prepared from different commercial caseins exhibit wide variations in consistency when mixed with a given proportion of water and also differ greatly in their subsequent behavior, notably in the interval 10 of time which may elapse between the initial mixing with water and the point at which the glue "sets", i. e., becomes too thick to spread. Various methods have been proposed to control this interval, generally termed the "life" 15 of the glue, such as the addition of animal glue or salts of the alkali or alkaline earth metals. The use of animal glue for this purpose is uneconomical, since its natural strength, which otherwise would contribute 20 to the adhesiveness of the mixture, depreciates considerably under these conditions. The addition to casein glues and adhesive compositions, of alkali metal phosphates, fluorides and other salts which by interaction 25 with lime liberate caustic alkalies is undesirable beyond a certain point; that is to say, any large excess of alkali over the amounts required to dissolve the casein and to impart a proper consistency and ultimate water-re- 30 sisting property to the glue or adhesive is to be avoided since the caustic alkali thus produced causes hydrolysis of the casein and consequent loss of strength.

We have now found that soybean meal 35 added to casein glues and adhesive compositions has a marked effect in retarding the "setting" thereof, thereby extending the life of such glues and adhesive compositions. As examples, the rates of change in the viscosity of a commercial casein glue (A') and of the same glue with respectively 7% (B), 15% (C) and 30% (D), of pulverized soybean meal added (in place of equivalent amounts of the casein) are compared below. 40 The values represent readings on the Stormer viscosimeter (provided with a 500 gram weight) at regular intervals after mixing, the conditions of making the four liquid glues A', B, C and D being identical in every 45 respect, except as to the addition or omis- 50

sion of the stated amounts of soybean meal.

The "commercial casein glue" here referred to was a mixture of dry casein, alkaline salts of sodium, sodium fluoride and hydrated lime, mixed together in proportions similar 55 to those described in the present application. The said commercial casein glue base and each of the composite glue bases referred to herein were mixed in every case with double their weight of water at approximately 60° 60 F., and the measurements of the viscosities of the glues thus prepared were made at a constant temperature of 70° F.

|    | 1 hr. | 3 hrs. | 5 hrs. | 7 hrs. | 9 hrs. | 11 hrs. | 13 hrs. | 65 |
|----|-------|--------|--------|--------|--------|---------|---------|----|
| A' | 26    | 9      | 2      | set    | 2½     | 2       | 1½      |    |
| B  | 30    | 24     | 11     | 5      | 7      | 4       | 3       |    |
| C  | 24    | 17     | 12     | 7      | 7      | 3       | 2       |    |
| D  | 22    | 14     | 10     | 9      | 7      | 6       | 6       |    |

In all the above tables it should be observed that the higher the reading, the lower the viscosity, and vice versa.

It will be understood that by varying the proportion of meal added, the life of the 75 glue can be controlled within wide limits. We prefer to use meal which has been ground to pass through a 120 mesh screen or finer, although a coarser product of approximately 80 mesh has given good results in casein 80 waterproof glues. With the finer meal a smoother glue is obtained.

By the term "80 mesh" as used above and in certain of the claims, we mean that the meal should be of such a degree of fineness as to 85 pass through an 80 mesh standard screen without leaving any substantial residue. The particles are not of uniform size. While the coarsest grains may approximate 80 mesh, it is obvious that, in the milling process, a 90 considerable proportion of the particles are reduced to much smaller dimensions.

In carrying out the invention the casein is mixed with an appropriate amount of the soybean meal, and to this mixture is added 95 an alkaline earth oxide or hydroxide with or without one or more water soluble alkali metal salts, preferably those which by themselves react alkaline to litmus and are capable of dissolving the casein and the pro- 100

teids of the soybean meal. The salts are such as react with hydrated lime, in the presence of water, to liberate caustic alkali, (e. g. caustic soda). It is well known that caustic alkali and alkaline-reacting salts of alkali metals both are capable (in the presence of water) of dissolving casein, and they both also can dissolve the proteids of the soybean meal. The alkali metal salts of alkaline character, the lime and the caustic alkali each have the property, in the presence of water of reacting upon casein, and the property of reacting upon the proteids of soybean meal. Hence when water is added to a mixture of such alkali metal salt (say sodium carbonate) lime, casein and soybean meal, the said salt will react with the lime, producing a caustic alkali and a precipitate of calcium carbonate, and (in the specific examples here given) leaving an excess of the lime, and both the caustic alkali and the excess of lime present and the water will then serve to react upon the casein and the proteids contained in the soybean meal. Likewise on adding water to a mixture of the casein, soybean meal and lime, the lime and water will react with the said proteids.

The following examples of mixes which have given satisfactory results when applied to joints and laminated woods will serve to define more particularly the character of the invention, but we do not desire to be limited to the particular compounds or proportions herein set forth. The parts are by weight.

In referring to an "alkaline earth oxide or hydroxide" we include, for the sake of convenience, the oxide and hydroxide of magnesium.

#### Example 1

Casein 60 parts; soybean meal (120 mesh) 10 parts; hydrated lime 15 parts; sodium fluoride 5 parts; sodium carbonate 5 parts; sodium phosphate 3 parts.

#### Example 2

Casein 35 parts; soybean meal 30 parts; hydrated lime 20 parts; sodium fluoride 4 parts; sodium carbonate 9 parts.

#### Example 3

Casein 50 parts; soybean meal 20 parts; hydrated lime 15 parts; magnesium oxide 5 parts; sodium fluoride 7 parts; trisodium phosphate 3 parts.

#### Example 4

Casein 40 parts; soybean meal 32 parts; hydrated lime 18 parts; sodium fluoride 2 parts; sodium carbonate 7 parts; sodium arsenate 1 part.

These examples indicate the dry materials which are mixed together to form the dry glue base. The dry mixture is to be subsequently incorporated with water by the

methods well known to users of casein glues. We prefer to use from 2 to 2½ parts of cold water to 1 part of the dry base. The water is put into a kettle provided with an efficient stirring device; the dry glue base (e. g. one of the above formulas) is added slowly and mixed thoroughly for about 20 minutes and is then ready for use.

The term "casein" is used herein in its usual meaning, to denote certain phospho-proteid matter contained in milk and skim milk, such as cows' milk, etc.

The soybean meal preferably used is the product obtained by grinding the cake left in the presses after expressing the major portion of the oil; it usually contains about 6 to 8% of residual oil. It will be understood that the further removal of oil by treatment of the press cake, or the direct extraction of the oil from the seed with suitable solvents (e. g. after crushing) are not precluded. The term "soybean meal" is intended to cover such products, as distinguished from soybean containing the full natural oil content.

The addition of soybean meal to casein glues, in place of the cottonseed meal and peanut meal as described and claimed in our application under Serial Number 99,423 is preferable in cases where a light colored glue is required, as the commercial meals of cottonseed and peanut contain natural coloring matters which detract from the appearance of the glues in which they are used. It is understood that in such cases we prefer to use meal from the light colored varieties of soybean, such as the Manchurian yellow, rather than the inferior blue and black varieties which yield darker glues.

The term "alkaline earth oxide" as used herein is intended to include the unhydrated as well as the hydrated oxides (hydroxides). The term "a salt" is intended to cover one or several salts.

No claim is made herein to the use of casein or to the use of soybean meal, alone, as the base of the adhesive, but to the joint use of these, whereby the "life" of the adhesive is prolonged. No claim is made to the use, with casein glues, of the extracted and reprecipitated soybean proteids, along with casein.

We claim:—

1. A dry glue base containing a quantity of casein, a smaller quantity of soybean meal and an alkaline earth oxide together with a water-soluble alkali metal salt which can react with lime in the presence of water to form caustic alkali and a precipitate, the said salt and alkaline earth oxide being in amounts sufficient for the reaction products and water to dissolve the casein and the proteids of the soybean meal, such base being adapted, upon mixing with water, to form an adhesive, which adhesive will have a longer period of workable viscosity than

would a similar composition without the soybean meal and with the casein correspondingly increased.

2. A new dry glue base containing casein, soybean meal and an alkaline earth oxide, the latter being in amount sufficient to react with the casein and the proteids in said soybean meal, such base being adapted upon mixing with water, to form an adhesive, 10 which adhesive will have a longer period of workable viscosity than would a similar composition without the soybean meal and with the casein correspondingly increased.

3. A new dry base for the manufacture of adhesive material comprising a quantity of casein, incorporated with a smaller quantity of soybean meal ground to pass an 80 mesh screen, and an alkaline earth oxide capable of, and in amount sufficient for reacting with 20 the casein and the proteids of the soybean meal, when water is added, such base being adapted, upon mixing with water, to form an adhesive, which adhesive will have a longer period of workable viscosity than would a similar composition without the soybean meal and with the casein correspondingly increased.

4. A new dry base for the manufacture of adhesive material comprising casein, incorporated with soybean meal ground to pass a 30 120 mesh screen, and an alkaline earth oxide capable of, and in amount sufficient for reacting with the casein and the proteids of the soybean meal, when water is added, such base being adapted, upon mixing with water, to form an adhesive, which adhesive will have a longer period of workable viscosity than would a similar composition without the soybean meal and with the casein correspondingly increased.

5. A new dry base for the manufacture of adhesive material comprising a quantity of casein, incorporated with a smaller quantity of soybean meal ground to pass a screen finer 45 than 120 mesh, and an alkaline earth oxide capable of, and in amount sufficient for reacting with the casein and the proteids of the soybean meal, when water is added, such base being adapted, upon mixing with water, 50 to form an adhesive, which adhesive will have a longer period of workable viscosity than would a similar composition without the soybean meal and with the casein correspondingly increased.

6. A new dry base for the manufacture of adhesive compositions, comprising casein incorporated with soybean meal ground to pass an 80 mesh screen, an alkaline earth oxide 60 and an alkali metal salt capable, in the presence of water, of dissolving the casein and the proteids of the soybean meal, the total amounts of such alkaline earth oxide material and of such alkali metal salt being sufficient, in conjunction with the soluble reaction products of the interaction thereof, to dissolve

the casein and the proteids of the soybean meal, and the amount of such casein being greater than the amount of such soybean meal, such base being adapted, upon mixing with water, to form an adhesive, which adhesive will have a longer period of workable viscosity than would a similar composition without the soybean meal and with the casein correspondingly increased. 70

7. A new dry base for the manufacture 75 of adhesive compositions, comprising casein incorporated with soybean meal from which a large part at least of the oil has been removed, ground to substantially all pass through an 80 mesh screen, and an alkali metal salt capable of dissolving the casein and the proteids of the soybean meal, together with an alkaline earth oxide, the said salt and oxide being in amounts, in conjunction with the reaction products formed, sufficient to dissolve the casein and the proteids of the soybean meal when water is added, such base being adapted, upon mixing with water, to form an adhesive, which adhesive will have a longer period of workable viscosity than would a similar composition without the soybean meal and with the casein correspondingly increased. 80 85

8. A new dry base for the manufacture of adhesive compositions comprising a quantity 90 of casein incorporated with a smaller quantity of soybean meal from which at least a part of the oil has been removed, ground to substantially all pass through an 80 mesh screen, and an alkaline alkali metal compound capable of dissolving the casein and the proteids of the soybean meal, when water is added, together with slaked lime, the said alkali metal compound and lime being in amount sufficient to dissolve the casein and the proteids of the soybean meal, such base being adapted, upon mixing with water, to form an adhesive, which adhesive will have a longer period of workable viscosity than would a similar composition without the soybean meal and with the casein correspondingly increased. 95 100

9. A dry glue base containing casein, soybean meal and an alkaline earth oxide, together with a water-soluble alkali metal salt 105 which can react with lime in the presence of water to form caustic alkali and a precipitate, the said salt and alkaline earth oxide being in amounts sufficient for the reaction products and water to dissolve the casein and the proteids of the soybean meal, such base being adapted, upon mixing with water, to form an adhesive. 110

10. A novel material in the glue art, the same being an intimate dry mixture of casein 125 and soybean meal, the former being in excess of the latter.

11. A novel material in the glue art, the same being an intimate dry mixture of casein and soybean meal, the amount of such casein 130

being substantially greater than the amount of protein contained in the soybean meal.

12. The method of producing a glue of comparatively long working life from a dry glue base including casein, a water-soluble alkali metal salt which is alkaline to litmus, and an alkaline earth metal oxide, which process comprises incorporating soybean meal in such dry glue base, and thereafter mixing this new glue base with water, the portion of the soybean meal used being sufficient to retard the setting of the glue produced by said admixture with water.

13. A dry glue base containing casein, soybean meal and lime, the latter being in amount sufficient to react with the casein and the proteins in said soybean meal.

In testimony whereof we affix our signatures.

20 LAWRENCE BRADSHAW.  
HENRY V. DUNHAM.

25

30

35

40

45

50

55

60

65